

G. A. HENDERSON,

VEGETABLE FIBER COMPOSITION AND PROCESS OF MAKING SAME.

APPLICATION FILED NOV. 30, 1915.

1,370,647.

Patented Mar. 8, 1921.



Witnesses  
A. A. Lybrand  
C. H. Dealer

Inventor  
George A. Henderson,  
Edgar W. Kitchin,  
his Attorney.

# UNITED STATES PATENT OFFICE.

GEORGE A. HENDERSON, OF ST. ALBANS, WEST VIRGINIA, ASSIGNOR TO T. S. CLARK,  
OF CHARLESTON, WEST VIRGINIA.

## VEGETABLE-FIBER COMPOSITION AND PROCESS OF MAKING SAME.

1,370,647.

Specification of Letters Patent.

Patented Mar. 8, 1921.

Application filed November 30, 1915. Serial No. 64,285.

To all whom it may concern:

Be it known that I, GEORGE A. HENDERSON, a citizen of the United States, residing at St. Albans, in the county of Kanawha 5 and State of West Virginia, have invented certain new and useful Improvements in Vegetable-Fiber Compositions and Processes of Making Same; and I do hereby declare the following to be a full, clear, and exact 10 description of the invention, such as will enable others skilled in the art to which it appertains to make and use the same.

The primary object in view is the effective impregnation of vegetable fiber with preservative material for producing a durable and efficient compound especially well adapted for paving and like purposes.

A further object in view is the expanding 20 of the voids or interstices of vegetable fiber by the actions of cooking, heating and treating the fiber, and of driving out the moisture therefrom closely followed by the introduction thereto of a preserving material of a binding nature whereby such fiber is caused 25 to be impregnated to its maximum capacity therewith.

These and other objects, such as will hereinafter in part be set forth and in part become obvious, are attained in the carrying 30 out of the process hereinafter specified, which process may most readily be disclosed in conjunction with a statement of operation of an apparatus especially adapted for the carrying out of the process, such as 35 illustrated in the accompanying drawings, in which,—

Figure 1 is a sectional elevation of such apparatus;

Fig. 2 is a cross section taken on the planes 40 indicated by line 2—2 of Fig. 1 and looking in the direction indicated by the arrows.

Fig. 3 is an enlarged, detail, fragmentary plan view of the conveyer belt and trough, parts of the belt being broken away for 45 disclosing the trough, and intermediate portions of each being broken out for the saving of space.

Referring to the drawing by numerals, 1 is a cooker or boiler, heated by steam pipes 50 2 and having a hopper bottom terminating in a discharge opening controlled by the rotary gate 3 which is adapted to deliver material from the container 1 into the trough 4 and onto the endless conveyer belt 5. At appropriate points in the length of

the trough 4 there are arranged presser rollers 6, 6 beneath which material from tank 1 is designed to be conveyed for having moisture expressed therefrom prior to the discharge of such material from the terminus of conveyer 5. The trough 4 and conveyer belt 5 are foraminated for allowing liquid, pulp and fine solids such as would produce impalpable powder to pass therethrough and to fall into a tank or container 60 7 arranged beneath the trough 4. A draining plate 8 extends from tank 7 for the balance of the length of trough 4 beyond the tank. Attached to the under side of cooker or boiler 1 may be a drainage pipe (not 70 shown) for removal of the sap and essences from the cooker from time to time.

A heater is provided consisting of a housing 9 having a stack or exhaust opening 9' at its upper portion and at its lower portion 75 having a gas or other appropriate furnace 10. Nested within the housing 9 is a hollow vat or container 11 which is spaced from the walls of the housing 9 and arranged just above the furnace 10 so that the products of combustion therefrom are designed to pass freely all about the container 11. The container or drum 11 is open ended, having an intake opening 12 at one end into which is delivered the materials discharging 80 from the end of the trough 4, which intake opening may be equipped with a rotary gate such as gate 3 in Fig. 1. Stationed between intake opening 12 and belt 5 and delivery chute 13 may be measuring 85 tanks for the purposes hereinafter described. At the other end of the container or drum 11 is placed a discharge opening for steam and fumes, as will hereinafter be pointed out.

A delivery chute 13 is provided for the preserving and adhesive material, such, for example, as asphalt, which is delivered, hot, that is in a molten condition, from container 14, which is heated in any appropriate manner. The chute 13 discharges into the drum 11 from the measuring tanks 14' and into the opening 12. A shaft 15 is journaled in the casing 9 and extends axially throughout the drum 11. Propeller blades 100 16 are carried by the shaft, said blades being fixed to the shaft at intervals along the same in position for slowly feeding the material within the drum along the same from the intake 12 toward the discharge end 110

thereof. Gearing 17 driven by motor 18 is provided for actuating the shaft 15 and its propellers. At the upper part of the discharge end of drum 11, the vapor discharge pipe 20 communicates with the drum, and a blower or fan 19 is arranged in pipe 20 and is adapted to be actuated for drawing steam or other gas from within the drum 11 and for effecting a forced discharge 10 thereof, thus tending to create a vacuum within the drum 11. A discharge chute 21 is arranged to receive material discharged from drum 11 and the end of the drum is formed with an opening for permitting discharge 15 of material into chute 21. A door 22 is adapted to close said opening whenever it is desirable to prevent discharge of material temporarily.

In carrying out my process, tank 1 is 20 supplied with water and maintained in a boiling condition. Vegetable materials are supplied to the tank and retained therein a length of time sufficient for exhausting sap, pith and all soft and pulpy substances from 25 the vegetable materials, so that the fibrous material is left with the pores or interstices expanded and cleared, but filled with water. The vegetable materials may be of such fibrous substances as straw, corn stalks or 30 sugar cane, but I prefer to employ the more nearly solid vegetable materials such as the hard-woods, the softest being chestnut. In instances where I use such hard wood as beech, quebracho, fustic, maple and like 35 woods of such density and close grain, I prefer to shear the logs into thin sheets, as hereinafter described, in which operation, as a modified procedure in my process, the logs of wood are boiled in water a predetermined 40 length of time before being sheared into sheets, then ground into particles as herein-after described, and in such instances I rely for expansion of the pores of the particles, and for thorough impregnation by a binding 45 preservative, upon first heating the particles, to expand them, then introducing the particles into a bath of hot asphalt, and maintaining them in such heated condition, until further expanded by such heat, and until 50 the open pores of the particles have become saturated with the asphalt or other preservative binder. Whatever the material, the vegetable substance is comminuted before introduction into the tank 1, and in the instances of the use of the harder woods, I 55 preferably rotate a log positioned in engagement with a knife for shearing off thin sheets, after the manner customary in making veneer, and then grind up the thin sheets 60 thus produced into fragments of irregular lengths and breadth, and say an average of a thirty-second of an inch in thickness. The comminuted particles are of uniform thickness but vary in length and breadth 65 quite materially, say from those the size of a

cube whose thickness is that of the particles up to three quarters of an inch in length, and approximately one quarter of an inch wide, the object of this operation being the uniform impregnation, and uniform heating 70 of each particle without interfering substantially with the grading of the particles, into various sizes from those the size of a cube whose thickness is that of the particles up to approximately three quarters of an inch 75 in length, by the use of screens, not shown in the drawings, so that the smaller particles will, as nearly as may be, fill the voids between the larger ones, thus insuring further density of the completed, compressed 80 product.

In the instance where the fibrous substances have their pores and interstices filled with water from the cooker, they are discharged by gate 3 onto belt 5, and the pulpy 85 substances removed from the fiber by boiling or saturation are delivered also onto belt 5. The fiber is carried along the belt and discharged into intake 12, but some of its moisture, impalpable dust and pulpy matter is 90 drained through the belt and trough 4 down into tank 7. The rollers 6 serve to express most of the moisture from the fiber before it enters intake 12, but this compressing action tends to close the pores or interstices of 95 the fibers, and I, therefore, provide for again expanding them by driving out from the fiber the remaining moisture by heating the fiber. This heating operation may be an independent step, but efficient results may 100 be secured by combining this step with that of impregnation with the preserving and adhesive material. To this end, the fibrous material is discharged directly from trough 4, preferably through measuring apparatus, 105 not shown, into intake 12, and, coming into contact with the hot material within, has its remaining moisture driven out, which results in expanding and opening the pores or interstices in the particles which had just 110 previously been somewhat contracted by the pressure rollers 6. Just as the moisture is discharging as steam from the fiber, the asphalt or other preservative and adhesive material in drum 11 enters the expanded and 115 expanding pores of the fibers and fills the same only in sufficient quantity to cause the fiber, (when subsequently contracted as hereinafter explained, and compressed) to become thoroughly saturated with the preserving 120 binder, and with just such excess thereof as may be sufficient to act as a binder of the impregnated and coated particles, care being taken that the percentage of preservative-binder shall be such that when the heated 125 mixture has been compressed, and the particles of fiber have been contracted to approximate normal size, as a result of the affinity of the molecules of asphalt or other heavy preservative, for, each other, during cooling, 130

there shall exist in the completed, compressed, cold product only sufficient preserving binder to completely fill the pores of the fiber, to coat the same, to fill the voids 5 between the particles, in their compressed condition, and to bind them to each other.

Hence, depending upon the character of the wood or other vegetable matter, and the impregnating and cementing agency selected, excellent results from my process are obtained by the adoption of the proportions of such particles and agencies, as follows: (the percentages, by volume being taken on the basis of the completed product), viz:

15 Preservative and binder, by volume ----- 25% to 40%  
Fibrous material, by volume ----- 60% to 75%  
Preservative and binder, by weight ----- 30% to 65%  
20 Fibrous material, by weight ----- 35% to 70%

These proportions can be accurately determined for any particular fiber by examination of the finished material, for determining 25 if the fiber is impregnated to its full capacity without, however, carrying excess or waste asphalt or like material. They may be likewise determined accurately by measuring first the voids and pores in the dry, uncontracted, uncompressed fiber, secondly the degree of contraction and compression, and thirdly adding sufficient quantity of preserving and binding material to bind the particles together after they have exhausted 35 their absorbing efficiency measured by their contracted, compressed size.

The materials are slowly but thoroughly agitated within the drum 11, and the steam discharging from the fibrous particles is 40 drawn out of pipe 20 by the action of the fan 19.

From time to time, door 22 is opened, and the hot material is run out through chute 21 to trucks for delivery to the previously constructed street base, where it is preferably 45 spread at a thickness of approximately twice the expected finished thickness. That is, for example, it may be spread three inches thick, and it is then rolled, by ordinary steam 50 rollers, down to approximately an inch and a half in thickness. In thus compressing the material, it is preferable to use a light steam roller, and then follow with a sufficiently heavy roller for completing the desired 55 amount of compression. The thus completed product may be finished off with any desired sealing or other coat.

In the event the material fed through the chute 21 is not to be used at once, it is preferable 60 to form the material into blocks of convenient size for handling, by slight compression applied to an ordinary baling press. The blocks thus produced may be stored for future use, and when used are broken up 65 manually or otherwise and then reheated to a

plastic state to facilitate spreading the same on the road base, or otherwise compressing the same into shape.

After the material is emitted, hot, from the chute 21, it may be mixed with asbestos, 70 sand, cement or other filler of a fireproof nature, or it may be subjected to a solution of fireproof nature, before the same has cooled; or, in the event the material is not to be used at once, after emission from the 75 chute 21 it may be baled as aforesaid, and then, after being broken up, it may be placed within a reheating machine, and in this operation, sand, cement, or other material may be added, to give the product added density, 80 if desired.

What I claim is:—

1. The herein described process of treating fibrous material which consists in subjecting the same to a cooking or boiling operation, removing the material from the cooker or boiler and extracting moisture from the material, then subjecting the material to the action of a hot binding and preservative agent in a vat to convert the remaining moisture in the material into steam and to impregnate the pores of the material with the binding and preservative agent, and finally removing the impregnated material 90 from the vat.

2. The herein described process of treating fibrous vegetable material which consists in subjecting the same to a cooking or boiling operation in the presence of water, for a pre-determined period, then removing 100 the material from the cooker or boiler, then while the material is hot extracting moisture from the same, then subjecting the material to the action of a hot binding and preservative agent in a vat to convert the remaining 105 moisture in the material into steam and to impregnate the pores made vacant by the escape of the moisture from the material with the binding and preservative agent, drawing the steam vapors out of the vat during said impregnation, and finally removing the impregnated material from the vat.

3. The herein described process of treating fibrous vegetable material, which consists in subjecting the same to a cooking or 110 boiling operation, removing the material from the cooker or boiler while hot, then extracting the moisture from the material while hot, then conveying the material through an open ended vat containing hot 115 binding and preservative agent to convert the remaining moisture in the material into steam and to impregnate the pores of the material with the binding and preservative agent, and drawing the steam vapors out of the vat during said impregnation.

4. The herein described process of treating fibrous vegetable material, which consists in subjecting the same to a cooking or 120 boiling operation, removing the material 125 from the vat during said impregnation.

from the cooker or boiler while hot, then extracting the moisture from the material while hot, then conveying the material through an open ended vat containing hot binding and preservative agent to convert the remaining moisture in the material into steam and to impregnate the pores of the material with the binding and preservative agent, drawing the steam vapors out of the vat during said impregnation, and finally compressing the material.

5. The herein described process which consists in moving fibrous material in a moist condition through hot asphalt in a vat so as to convert the moisture in the material into steam and to impregnate the material with the asphalt during the movement of the material through the asphalt, drawing the steam vapors out of the vat during 10 said impregnation, and after the material has been moved through the hot asphalt and before the impregnated material cools subjecting the same to pressure.

6. In a process of treating fibrous vegetable material, forming comminuted fibrous particles of substantially uniform thickness, of irregular lengths and breadths, removing sap, soft, pulpy portions and all matter soluble in water, from the particles, and impregnating the particles with a preserving compound of a binding nature, and compressing the same into shape.

7. In a process of treating fibrous vegetable material, forming comminuted fibrous particles of exactly uniform thickness but of irregular lengths and breadths, expanding the particles by heat, extracting all moisture from the particles by conveying the same through an open ended vat containing hot binding and preservative agent to expand the pores of the fiber, and to convert the remaining moisture in the particles into steam and to impregnate the pores of the material with a pre-determined quantity 45 of binding preservative agent, drawing the steam vapors out of the vat during said impregnation, and then compressing the material into shape.

8. In a process of treating fibrous vegetable material forming comminuted fibrous particles of hard wood of exactly uniform thickness, but of irregular lengths and breadths, grading the sizes of said particles from just larger than impalpable dust up to 55 three quarters of an inch in length, and mixing percentages of each size of said particles so that the smaller ones will, as nearly as may be, fill the voids between the larger particles; then conveying the same through 60 an open ended vat to heat the same, then depositing the same into a hot binding preservative agent within the vat, and agitating the same a sufficient length of time to expel from the particles all remaining moisture, and to abnormally enlarge and expand

the pores of the particles, to impregnate the same with a pre-determined quantity of binding preservative agent, only sufficient in quantity to completely fill the pores within the fibrous particles, in their subsequently contracted compressed condition, to surround the particles, and fill the voids between the same, in their completed product, and to bind the same together; then while hot, removing the material from the vat, and while cooling compressing the same into shape.

9. In a process of treating fibrous vegetable material, forming comminuted fibrous particles of substantially uniform thickness, but of irregular lengths and breadths, subjecting the same to a cooking or boiling operation, removing the material from the cooker or boiler, then extracting the moisture from the material while hot, then conveying the material through an open ended vat containing hot binding and preservative agent, to convert the remaining moisture in the material into steam and to impregnate the pores of the material with the binding and preserving agent, drawing steam vapors out of the vat during said impregnation, and finally mixing mineral matter with the impregnated vegetable matter while the same is hot, and pressing the same into shape.

10. The herein described process of treating fibrous vegetable matter, which consists in subjecting the same to a cooking or boiling operation, removing the material from the cooker or boiler, removing the sap and matter soluble in water loosened from the material in the boiler from the boiler, then compressing the material to further remove its moisture content, then conveying the material through an open-ended vat containing hot binding and preservative agent, deposited on the fibrous material in pre-determined quantities of each, then agitating the mixture in the presence of heat to the extent of expelling and expressing all remaining moisture from the vegetable fiber, drawing out of the vat all steam and vapors from the expanded fibers pores and surfaces, simultaneously impregnating the pores of the material with a predetermined quantity of preservative and binding agency, sufficient to fill the pores and voids in and between the particles; then removing the mixture from the vat; then allowing the material to cool; then reheating the material, then mixing a pre-determined quantity of sand and then compressing the mixed material into shape, substantially as described.

11. In a process of treating fibrous vegetable material, forming comminuted fibrous particles, clearing the pores or interstices of the particles of sap and like soft materials, expanding the pores by heat, impregnating the expanded pores, while expanding, with a preservative compound of a

binding nature; then contracting the particles by cooling the mass; then reheating the material; then compressing the same, while hot, into shape.

5 12. A fibrous composition, comprising vegetable fiber which has been cleared of sap and soft substances from its pores, and impregnated with preserving material, the fiber being in the form of comminuted par-

ticles of substantially uniform thickness, 10 and irregular lengths and breadths.

In testimony whereof I affix my signature in presence of two witnesses.

GEORGE A. HENDERSON.

Witnesses:

J. RICE WARRICK,  
J. S. TEAY.